

April 29, 1969

P. E. THOMA

3,440,881

HUMIDITY SENSING ELEMENT

Filed Sept. 27, 1967



Fig. 1.



Fig. 2.

Fig. 3.



Fig. 4.



Fig. 5.

INVENTOR

PAUL E. THOMA  
BY

Andrus & Stark  
Attorneys

**1**

3,440,881

**HUMIDITY SENSING ELEMENT**

Paul E. Thoma, Milwaukee, Wis., assignor to Johnson Service Company, Milwaukee, Wis., a corporation of Wisconsin

Filed Sept. 27, 1967, Ser. No. 671,067

Int. Cl. G01n 25/56

U.S. Cl. 73—337.5

12 Claims

**ABSTRACT OF THE DISCLOSURE**

The invention relates to a synthetic, variable dimension, humidity sensing element including a core or base formed of a crosslinked material produced by the reaction of a compound containing glucoside chains and a stabilizing monomer capable of reacting with the hydroxyl groups of the glucoside. Bonded to at least one surface of the core is a moisture sensitive organic material which can either be a noncrosslinked compound containing glucoside chains or a partially crosslinked reaction product of a compound containing glucoside chains and a monomer capable of reacting with the hydroxyl groups of the glucoside.

The crosslinked core provides resistance to creep, while the outer layer provides toughness for the element.

Humidity sensing devices are generally classified as a mechanical type or an electrical type. The mechanical type of humidity sensing device utilizes the dimensional change which occurs in the humidity sensing material when there is a change in relative humidity to either indicate the relative humidity or to actuate a humidity control system, while the electrical type utilizes a change in the electrical resistance or capacitance of the humidity sensing element due to a change in relative humidity.

The common forms of a naturally occurring humidity sensing element, such as human hair, wood, gold beater's skin, and animal horn, have certain inherent disadvantages. The elements are extremely fragile and frequently are damaged in shipment. More important, however, the elements are difficult to produce and this is particularly true of the horn element, for it requires a very precise operation to cut the horn material into thin layers of uniform thickness. Since most of the conventional elements are naturally occurring, it is difficult to obtain uniform performance from element-to-element and uniformity is only obtainable through very careful calibration. Moreover, the elements generally do not retain their original calibration after long term exposures to extremes of humidity and in many cases require frequent re-calibration.

Another disadvantage of some conventional varying dimension humidity sensing elements is that the elements are difficult to clean, for they cannot satisfactorily be washed with solvents or detergent solutions without adversely affecting their performance. In view of this, the elements must be replaced after a period of use as they cannot readily be cleaned.

To overcome the disadvantages of the natural occurring materials, there have been attempts in the past to use synthetic humidity sensing materials. Many of these synthetic materials, however, undergo creep when stressed. The stresses develop as the result of film production, or as the result of moisture concentration variations within the film, or when tensile force is applied to the element to keep the element taut. The resulting reaction to these internally and externally developed stresses results in creep of the film which causes set point and sensitivity changes.

The present invention is directed to a synthetic, vary-

**2**

ing dimension, humidity sensing element which has improved resistance to creep when stressed and has improved chemical resistance. More specifically, the humidity sensing element of the invention includes a core or base formed of a crosslinked material produced by the reaction of a compound containing glucoside chains and a stabilizing monomer capable of reacting with the hydroxyl groups of the glucoside. Bonded to at least one surface of the core is a moisture sensitive, organic layer formed of a material having glucoside chains, such as cellulose or cellulose derivatives. In some cases the material of the outer layer can be partially crosslinked with a monomer capable of reacting with the hydroxyl groups of the glucoside.

5 The crosslinked core provides resistance to creep when the element is subjected to stress. The outer layers are sensitive to moisture, and as they are not fully cross-linked materials, provide toughness for the element, making the element less brittle than an element composed entirely of a crosslinked material.

10 The element of the invention has improved thermal stability and chemical resistance due to the crosslinking and can be washed with commercial solvents or detergent solutions without danger of destroying the performance of the element.

15 The humidity sensing element has a rapid response to humidity conditions and is not affected by extremes of humidity or temperature. The element has very little hysteresis and is substantially more stable than naturally occurring humidity sensing elements used in the past.

20 As the element is a synthetic product, it can be fabricated under controlled conditions and therefore requires less calibration from element-to-element.

25 Other objects and advantages will appear in the course of the following description.

30 The drawings illustrate the best mode presently contemplated of carrying out the invention.

In the drawings:

35 FIG. 1 is a fragmentary perspective view of the humidity sensing element of the invention;

40 FIG. 2 is a perspective view of the humidity sensing element in the form of a loop;

45 FIG. 3 is a perspective view of another modified form of the invention in which the element is in the form of a strip;

50 FIG. 4 is a diagrammatic view showing the use of the element in a mechanical-type humidity control system; and

55 FIG. 5 is a diagrammatic view showing the use of the element in an electrical-type humidity control system.

60 FIG. 1 illustrates a humidity sensing element 1 comprising a core or base 2, and outer layers 3 are integrally bonded to opposite surfaces of the core.

65 The core 2 is a substantially fully crosslinked reaction product formed by the reaction of a compound containing glucoside chains, such as a cellulosic material, and a stabilizing monomer capable of reacting with the hydroxyl groups of the glucoside. For example, the reactant can be cellulose or a cellulose ester in which the esterifying acids contain up to 20 carbon atoms and preferably up to 6 carbon atoms. Specific examples are cellulose triacetate, cellulose butyrate, cellulose propionate, cellulose succinate, cellulose phthalate or the like. Cellulose nitrate can also be used as well as mixed cellulose esters such as cellulose acetate-butyrate and cellulose acetate-propionate. Cellulose ethers in which the etherifying alcohol contains up to 8 carbon atoms, such as ethyl cellulose, methyl cellulose, hydroxypropylmethylcellulose, and hydroxybutylmethylcellulose can also be employed.

70 The stabilizing reactant which is crosslinked with the glucoside-containing compound can take the form of

monomers or partial polymers of urea-formaldehyde, phenol-formaldehyde, melamine-formaldehyde, triazine-formaldehyde, hexamethoxymethylmelamine, glyoxal, 2-hydroxy-adipaldehyde and the like.

The amount of the stabilizing monomer to be used in conjunction with the glucoside derivative can vary depending on the nature of the monomer. In the case of a resin which will crosslink with itself such as urea-formaldehyde, the monomer or partial polymer can vary within wide limits. Any excess of the monomer, over and above that which will react and crosslink with the glucoside will crosslink with itself. However, the stabilizing monomer should react with at least about 1% of the available hydroxyl groups of the glucosides and preferably with substantially all the available hydroxyl groups. With a stabilizing monomer or partial polymer that will not crosslink with itself, such as hexamethoxymethyl-melamine, the monomer should be used in a stoichiometric amount with the glucoside derivative or cellulosic material, or slightly less than a stoichiometric amount, for any excess will tend to act as a plasticizer for the core 2 and thereby increase the creep of the element.

To accelerate the crosslinking reaction, a catalyst is usually added to the reaction mixture. Any conventional catalyst for the particular monomers or partial polymers being employed can be used. For example, catalysts to be used with urea-formaldehyde, phenol-formaldehyde and melamineformaldehyde monomers include trifluoroacetic acid, methanesulfonic acid, monobutyl acid orthophosphate, n-butyl acid phosphate, p-toluenesulfonic acid, and the like.

In addition to the catalyst, it may also be desirable in many instances to employ a catalyst stabilizer which serves to tie up the catalyst until the crosslinking reaction is desired to occur. The catalyst stabilizers are conventional materials and include epoxide monomers and triethylamine, 2-dimethylaminoethanol, 2-diethylaminoethanol, and other volatile organic amines having boiling points below 250° C. The epoxide monomers can be used as both a catalyst stabilizer and as a reactant in the crosslinking reaction.

The outer layers 3 are preferably formed of a non-crosslinked compound containing glucoside chains, such as cellulose, a cellulose ester, or a cellulose ether. With the use of cellulose esters, the esterifying acids contain up to 20 carbon atoms and preferably up to 6 carbon atoms. Specific examples of cellulose esters are cellulose triacetate, cellulose butyrate, cellulose propionate, cellulose succinate, cellulose phthalate, cellulose acetate-butyrate, cellulose acetate-propionate, and the like. Cellulose nitrate can also be utilized.

When using cellulose ethers, the etherifying alcohol contains up to 8 carbon atoms and specific examples are ethyl cellulose, methyl cellulose, hydroxypropylmethylcellulose, hydroxybutylmethylcellulose and the like.

In some cases, the outer layers 3 can be formed of the partially crosslinked reaction product of a compound containing glucoside chains and a monomer or partial polymer capable of reacting with the hydroxyl groups of the glucoside. If the glucoside-containing compound of the outer layers 3 is partially crosslinked, the stabilizing reactant can take the form of monomers or partial polymers similar to those described in connection with the formation of the core 2. The amount of the stabilizing monomer to be used in conjunction with the glucoside derivative can vary, but it is important that only a partial crosslinking be obtained in order that the outer layers 3 will be flexible and tough. Thus, the amount of monomer to be used should be less than the stoichiometric amount required to completely crosslink with the hydroxyl groups of the glucoside. It is preferred that the crosslinking monomer or partial polymer be used in an amount such that less than 50% of the hydroxyl groups of the glucoside will be tied up by the crosslinking reaction.

As discussed with the formation of the core 2, a catalyst is usually added to the crosslinking reaction mixture and in some instances it may be desirable to also add a catalyst stabilizer such as that previously described.

The outer layers 3, whether non-crosslinked or partially crosslinked, should have a moisture sensitivity such that the outer layer will show a dimensional increase of at least 1% and preferably a 1½% to 7% with a change from 0% to 100% humidity. These sensitivity values are based on the outer layer dissociated from the core and need be in only one direction. In some cases the core 2 will be less moisture sensitive than the outer layers 3, while in other instances the core can have substantially the same moisture sensitivity as the outer layers or greater moisture sensitivity than the outer layers.

The thickness of the core 2 has a definite relation to the thickness of the outer layers 3. If a relatively moisture insensitive core is used and is too thick with respect to the thickness of the outer layers, the outer layers cannot provide the necessary dimensional change under changes in atmospheric moisture to deform the core. For an element having normal response, the thickness of the core will generally be in the range of about 0.1 to 5 mils, while the thickness of the outer layers 3 will be less than about 3 mils and should generally be between 10 to 400% of the thickness of the core 2. However, this relationship can vary depending on the moisture sensitivity and the modulus of elasticity of the outer layers 3 and core 2 and the response desired. The optimum thickness ratio of the outer surface layer with respect to the core 2 is generally arrived at experimentally.

It is preferred that the core 2 and outer layers 3 be co-extensive in length and width. However, in some instances, either the core 2 or the outer layers 3 may project beyond the other member of the element, and the function of the element will not be altered provided mechanical clamping of the element in use should be made directly to that area of the composite film containing the core and outer layers.

As shown in FIG. 1, the moisture sensitive layers 3 are bonded to opposite surfaces of the core 2, and as the core 2 and layers 3, or in some cases only the outer layers 3, change dimension in accordance with variations in relative humidity, the element will extend and contract linearly. However, it is contemplated that the moisture sensitive layers 3 need only be applied to one surface of the core 2, in which case variations in relative humidity will cause the element to bow or deflect, rather than moving linearly.

The core and outer layers 3 are bonded together throughout their dimensions and various methods may be employed to provide the bond between the members. For example, the outer layers 3 can be applied by coating the core 2 with a solvent solution of the reactants and subsequently evaporating the solvents and heating the laminated structure to achieve the crosslinking reaction. Alternately, the outer layers 3 can be bonded to the fully polymerized or crosslinked core 2 by use of auxiliary adhesives.

The sensitivity of the humidity sensing element can be further increased by hydrolyzing the outer surface of the cellulosic outer layer 3 to regenerated cellulose. The cellulosic outer layer 3 can be subjected to the influence of either an alkaline or an acid medium to hydrolyze substantially all of the acid radicals in the surface layer to thereby obtain a regenerated cellulose film which provides maximum moisture sensitivity. The hydrolyzation can be accomplished by dipping the element into an alkaline or acid bath and maintaining it in the bath for a period of time sufficient to hydrolyze the acid groups on the surface of the outer layers 3. Alkaline materials which can be employed for the hydrolyzation are aqueous or alcoholic solutions of alkali metal bases, such as sodium hydroxide, potassium hydroxide, or lithium hydroxide. Alternately, alcoholic solutions of strong organic bases, such

as tetramethylguanidine, trimethylamine, or benzyltrimethylammonium hydroxide can be used for the hydrolyzing action.

Hot alkaline solutions are preferred to increase the reaction rate. The time of contact or immersion in the alkaline solution depends, of course, on the material used, the temperature, and strength of the solution. For example, a two-hour hydrolysis period, using a 5% sodium hydroxide solution, was required to hydrolyze a mixed cellulose ester outer layer 3 to obtain the desired high sensitivity. By increasing the strength of the solution to 50%, an almost immediate hydrolyzation occurred. The most effective reaction conditions were found to be obtained by immersing the element in 230° F., 40% sodium hydroxide solution for 1 to 4 minutes, depending on the 15 desired layer thickness of the hydrolyzed layer.

After the hydrolyzation, the element is preferably rinsed in water to remove and dilute the alkaline residue.

Solutions of mineral acids, such as hydrochloric acid and sulphuric acid, can also be used to hydrolyze the 20 cellulose outer layer 3. However, the use of alkaline material provides a faster hydrolyzation and is preferred.

The preferred method of preparing the humidity sensing element is to initially dissolve the components of one of the outer layers 3 in a solvent, such as acetone, ethyl 25 acetate, ethylmethyl ketone, butyl alcohol, methylene chloride, nitroethane, cyclohexanone, ethylene dichloride, methylisobutylketone, isobutylacetate, hexane, toluene, diethyl ether, water, ethyl alcohol, xylene, isopropyl alcohol, or the like. It is preferred to dissolve the materials in the solvent or solvent mixture in a closed container with mixing or agitation. The solution is then cast onto a glass plate with an adjustable strike-off bar. After the solvent has evaporated to form the first outer layer 3, a solvent 30 solution of the core material is then cast over the dried first outer layer by use of the strike-off bar.

The solvent solution of the core material contains the glucoside compound and the stabilizing monomer along with the catalyst and the catalyst stabilizer.

When the solvent solution of the core material is cast 40 onto the first outer humidity sensitive layer, the solvents will partially dissolve the surface of the previously cast outer layer and when the solvent of the core solution is evaporated, an adherent bond is provided between the two layers.

Following the drying of the core 2, a solvent solution of the second outer layer is cast over the dried core. Again, the solvent will tend to dissolve the surface of the dried core, and when the solvent is evaporated, an adherent bond results between the core 2 and the second moisture 50 sensitive layer 3.

After the three-layer film is dry, the core 2, and in some cases the moisture sensitive layers 3, are polymerized or crosslinked by heating the laminated film on the glass plate to a temperature in the range of 200° to 400° F. 55 and preferably 250° to 375° F. for a period of time sufficient to crosslink the stabilizing monomer with the hydroxyl groups of the glucoside chains.

While the crosslinking or polymerization reaction can be made to occur at room temperature with most formulations, better results are obtained when the reaction is carried out at an elevated temperature.

Specific examples of solvent solution formulations for the outer moisture sensitive layer 3 and core layer 2 are as follows in weight percent.

#### EXAMPLE NO. 1

(A) Outer layer solution—uncrosslinkable:

10.00% cellulose acetate butyrate (17% combined butyryl)

90.00% ethyl acetate

(B) Crosslinkable core solution:

6.20% cellulose acetate butyrate (26% combined butyryl)

6.18% urea-formaldehyde (crosslinking material)  
1.60% triethylamine (catalyst stabilizer)  
0.15% p-toluenesulfonic acid (catalyst)  
2.21% n-butyl alcohol  
2.06% ethyl alcohol  
40.60% diacetone alcohol  
41.00% ethyl acetate

#### EXAMPLE NO. 2

10 (A) Outer layer solution—uncrosslinkable:  
10.00% cellulose acetate butyrate (37% combined butyryl)  
90.00% methylene chloride  
(B) Crosslinkable core solution:  
5.20% cellulose acetate butyrate (37% combined butyryl)  
5.58% urea-formaldehyde (crosslinking material)  
1.60% triethylamine (catalyst stabilizer)  
0.15% p-toluenesulfonic acid (catalyst)  
2.01% n-butyl alcohol  
1.86% ethyl alcohol  
33.60% diacetone alcohol  
50.00% methylene chloride

#### EXAMPLE NO. 3

(A) Outer layer solution—partially crosslinkable:  
10.00% cellulose acetate (39.4% acetyl)  
1.00% hexamethoxymethylmelamine (crosslinking material)  
1.60% 2-amino-2-methyl-1-propanol (catalyst stabilizer)  
0.05% p-toluenesulfonic acid  
0.05% n-butyl alcohol  
7.00% methylene chloride  
12.00% diacetone alcohol  
68.30% acetone  
(B) Crosslinkable core solution:  
10.00% nitrocellulose (10.9 to 11.2% nitrogen)  
1.50% hexamethoxymethylmelamine (crosslinking material)  
0.05% p-toluenesulfonic acid (catalyst)  
4.30% isopropyl alcohol  
0.05% n-butyl alcohol  
14.10% isobutyl acetate  
16.00% ethyl acetate  
14.00% 2-heptanone  
40.00% methyl ethyl ketone

#### EXAMPLE NO. 4

(A) Outer layer solution—uncrosslinkable:  
10.00% ethyl cellulose (45.5 to 46.8% ethoxyl content)  
90.00 methylene chloride  
(B) Crosslinkable core solution:  
8.00% ethyl cellulose (45.5 to 46.8% ethoxyl content)  
3.00% melamine-formaldehyde (crosslinking material)  
1.60% 2-dimethylaminoethanol (catalyst stabilizer)  
0.15% p-toluenesulfonic acid (catalyst)  
1.15% n-butyl alcohol  
1.00% xylene  
85.10% methylene chloride

A specific example of preparing the humidity sensing element of the invention is as follows:

The outer layer solvent solution shown in Example No. 1 was cast on a clean glass plate with an adjustable strike-off bar. After evaporation of the solvent, the solvent solution of the core material shown in Example No. 1 was then cast on the dried first outer layer by means of the strike-off bar. Following the evaporation of this solvent, the outer layer solution of Example No. 1 was then cast on the dried core with the strike-off bar to provide the second moisture sensitive layer. On evaporation of the solvent, a three-layer laminate was produced with each outer

layer having a thickness of about 0.3 mil and the core having a thickness of about 0.4 mil.

The composite structure, while on the glass plate, was heated to a temperature of 350° F. for 12 minutes to crosslink the cellulose acetate butyrate and the urea-formaldehyde monomer. The resulting laminate was cut into strips and the strips, when employed as humidity sensing elements, showed high sensitivity to moisture, excellent resistance to creep when subjected to stress and were resistant to chemical attack.

FIG. 2 shows a form of the invention in which the humidity sensing element 4, similar in construction to element 1, is in the shape of a loop. In this embodiment, the ends of the looped element 4 are disposed around rollers or supports 5 and mounting brackets 6 are attached to the rollers and serve to connect the rollers to a supporting structure. In service, the looped element is subjected to tensile stress, as for example, by providing a spring-loaded connection between one of the brackets 6 and the supporting structure. A variation in relative humidity will cause the element 4 to expand or contract in a linear or longitudinal direction to thereby produce a condition which can be used to indicate either the degree of moisture in the atmosphere or to actuate a humidity control device.

FIG. 3 illustrates a second modified form of the invention in which the element 7, similar in structure to element 1, is in the form of a strip. The ends of the element 7 are secured to clamps 8 which are connected to a supporting structure. As in the case of the element shown in FIG. 2, variations in moisture content in the atmosphere will cause the element 7 to expand and contract linearly and the expansion and contraction can be utilized in a conventional manner to provide an indication of the moisture in the atmosphere.

FIG. 4 is a schematic representation showing a simple, mechanical-type humidity indicator utilizing the element 7. In this embodiment, one end of the element 7 is permanently anchored to a fixed support 9, while the opposite end of the element is attached to a pointer 10 which is pivotally mounted at 11 and is adapted to move along a scale 12. The sensing element 7 is held under tension by a spring 13 attached to support 14. With this arrangement, the linear expansion and contraction of the element 7 will tend to pivot the pointer 10 and provide relative humidity readings on the calibrated scale 12.

FIG. 5 illustrates an electrical-type humidity indicator in which one end of the element 7 is permanently fixed to a support 15 and the opposite end of the element is connected to an indicator 16, and is under tension by a spring 17 attached to support 18. The indicator 16 is pivotally mounted at 19 and the opposite end of the indicator is provided with a wiper arm 20 which is adapted to move across a variable resistance element 21 connected in an electrical circuit with an ammeter 22 and a source of power 23. Changes in dimension of the element 7 serve to move the wiper arm 20 along the resistance element 21 to vary the current flow and thereby provide an indication of the humidity by the calibrated ammeter at the location of the sensing element or at a remote location. Alternately, the varying current in the circuit produced by changes in dimension of the element 7 may be used as an input signal to humidity control equipment.

The humidity sensing element of the invention, when under tensile stress, has improved resistance to creep and will thereby retain its set point and sensitivity to humidity changes throughout substantial periods of service without need for calibration.

The outer layers 3 provide an improved degree of sensitivity, as well as toughness for the element, enabling it to be subjected to substantial tensile stress without fracture or cracking.

Due to the crosslinked structure of the core 2, and in some instances the partially crosslinked structure of the moisture sensitive layers 3, the element is more resistant to solvents and detergents than conventional elements and

thus can be washed or cleaned with solvents or detergent solutions without destroying the performance of the element.

As the element is fabricated synthetically under controlled conditions, the characteristics of the element are 5 more uniform and less element-to-element calibration is required.

I claim:

1. A synthetic humidity sensing element, comprising a first layer, and a second layer extending over a substantial portion of surface of said first layer and bonded thereto, said first layer being the substantially fully cross-linked reaction product of a compound containing glucoside chains and a stabilizing monomer or partial polymer capable of crosslinking with the hydroxyl group of said glucoside chains, and said second layer being selected from the group consisting of (a) a non-crosslinked compound containing glucoside chains, and (b) a partially crosslinked reaction product of a compound containing 10 glucoside chains and a stabilizing monomer or partial polymer capable of crosslinking with the hydroxyl groups of said glucoside chains, said crosslinked first layer acting to prevent creep of the element and said second layer providing toughness for the element.
2. The element of claim 1 and including a third layer disposed on the outer surface of said second layer and composed of regenerated cellulose.
3. The element of claim 1 wherein said compounds are cellulosic materials.
4. The element of claim 1 in which said compounds are cellulose esters in which the esterifying acid contains up to 20 carbon atoms.
5. The element of claim 1, in which said monomers are selected from the group consisting of urea-formaldehyde, phenol-formaldehyde, melamine-formaldehyde, triazine-formaldehyde and hexamethoxymethylmelamine.
6. The element of claim 1, in which said compound of said second layer is a cellulose derivative, and said element includes a third layer bonded to the outer surface of said second layer, said third layer being produced by the hydrolyzation of said cellulose derivative and consisting essentially of cellulose.
7. A humidity sensing element, comprising a core being the substantially fully crosslinked reaction product of a compound containing glucoside chains and a stabilizing monomer or partial polymer capable of crosslinking with the hydroxyl groups of said glucoside chains, and outer moisture sensitive layers bonded to opposite surfaces of said core, said outer layers being selected from the group consisting of (a) a non-crosslinked compound containing glucoside chains, and (b) a partially cross-linked reaction product of a compound containing glucoside chains and a stabilizing monomer or partial polymer capable of crosslinking with the hydroxyl groups of said glucoside chains.
8. The element of claim 7 wherein said compound is cellulose or a cellulose derivative.
9. The element of claim 7 in which the monomer or partial polymer is selected from the group consisting of urea-formaldehyde, phenol-formaldehyde, melamine-formaldehyde, triazine-formaldehyde and hexamethoxymethylmelamine.
10. In a humidity sensing device, a humidity sensing element comprising a core being the substantially fully crosslinked reaction product of a compound containing glucoside chains and a stabilizing monomer or partial polymer capable of crosslinking with the hydroxyl groups of said glucoside chains, and outer moisture sensitive layers bonded to opposite surfaces of said core, said outer layers being selected from the group consisting of (a) a non-crosslinked compound containing glucoside chains, and (b) a partially crosslinked reaction product of a compound containing glucoside chains and a stabilizing monomer or partial polymer capable of crosslinking with the hydroxyl groups of said glucoside chains, means for con-

necting one end of said element to a fixed object, and means for applying tensile stress to the opposite end of said element.

11. The element of claim 1, wherein said second layer shows a dimensional increase greater than 1% with a change in relative humidity from 0% to 100%.

12. The element of claim 1, wherein the first layer has a thickness of 0.1 to 5 mils and the second layer has a thickness of 10% to 400% of the first layer.

5 2,604,423 7/1952 Slotterbeck et al. ---- 73—337 X  
3,295,088 12/1966 Smith ----- 73—335 X  
3,301,057 1/1967 Smith et al. ----- 73—337

## References Cited

## UNITED STATES PATENTS

LOUIS R. PRINCE, *Primary Examiner.*  
JOSEPH W. ROSKOS, *Assistant Examiner.*